

# UNITED STATES PATENT OFFICE.

SAMUEL MANSFIELD JONES AND IVAN OTHMA HARLOW, OF NORTH ADAMS, MASSACHUSETTS, ASSIGNORS TO ARNOLD PRINT WORKS, OF NORTH ADAMS, MASSACHUSETTS, A CORPORATION OF MASSACHUSETTS.

## MERCERIZATION.

1,392,833.

Specification of Letters Patent.

Patented Oct. 4, 1921.

No Drawing.

Application filed June 21, 1921. Serial No. 479,414.

To all whom it may concern:

Be it known that we, SAMUEL MANSFIELD JONES and IVAN OTHMA HARLOW, both, respectively, citizens of the United States, and residents of North Adams, in the county of Berkshire and State of Massachusetts, have jointly invented new and useful Improvements in Mercerization, of which the following is a description.

10 In the process of mercerizing cellulosic fibers of natural growth, such as cotton and linen, when these are interwoven or otherwise intermingled with filaments of artificial silk known as viscose, certain methods of 15 protecting such viscose filaments from deleterious attack by the caustic alkali employed for mercerization have been already set forth and claimed in United States patents to Samuel Mansfield Jones numbered and 20 dated respectively, 1,316,958, September 23, 1919; 1,343,138 and 1,343,139, June 8, 1920; 1,346,802 and 1,346,803, July 13, 1920.

The methods thus patented for protecting the viscose have consisted in the modification of the mercerizing caustic alkali solution by the addition thereto of either monohydric alcohol or formic aldehyde or phenol or glycerin or monacetin, each of which is an oxy-hydro-carbon compound belonging to 30 that division of chemistry commonly designated as organic; but we have discovered that the modification of the mercerizing caustic alkali solution by the addition thereto of certain salts having inorganic bases may 35 be made to accomplish similar useful results; and our present invention consists essentially in employing for this purpose such a salt of an inorganic base as when introduced into an aqueous solution of caustic alkali suitable for mercerizing cellulosic fibers, will not by reaction of the caustic alkali therewith undergo change of chemical composition but will be soluble in the 40 caustic alkali solution of standard strength 45 for ordinary mercerization to an amount not much less and preferably more than twenty per centum of this solvent. The salt of this constitution and capacity is to be dissolved to the full extent of its solubility in 50 the mercerizing caustic alkali solution which it is thus employed to modify.

The salts of most of the metals, even including the salts of magnesium and of the metals of the alkaline earths, when intro-

duced into an aqueous solution of caustic 55 alkali of suitable strength for ordinary mercerization will respectively, by reaction of the caustic alkali therewith, be converted into hydroxids of their metal bases or undergo further transformation into other 60 salts, neither of which, either because of its change of chemical composition or because of its practical insolubility, is capable of modifying such caustic alkali solution so as to accomplish the intended object of this 65 invention. Our investigations have shown, however, that all the salts of sodium, potassium and ammonium, whether formed with inorganic acids or with organic acids embraced in the aliphatic category, or in other 70 words the salts of what may be termed inorganic alkali bases, are more or less soluble in the standard mercerizing caustic alkali solution, and, when dissolved in this solution to the full extent of their respective 75 solubilities therein, tend in greater or lesser degrees to modify it in the direction of protecting the viscose silk intermixed with the cellulosic fibers to be mercerized against the injurious attack of the caustic alkali; but 80 that the injury resulting from such attack is only partially counteracted and is too considerable for economic requirements if the solubility of these modifying salts is in any case much below twenty per centum of 85 the weight of the solvent constituted by the standard mercerizing caustic alkali solution; and that in order to obtain an entirely satisfactory protection of the viscose silk under the conditions indicated this percentage 90 should be exceeded.

Among the salts which are soluble to the extent thus specified as practically available for the purposes of the present invention the following may be mentioned as 95 typical, to wit: sodium nitrite, sodium formate, sodium citrate, sodium lactate, potassium sulfite, potassium formate, potassium acetate, potassium citrate and ammonium citrate; but the best of these has proved to be 100 potassium acetate which when introduced into the standard caustic alkali solution for ordinary mercerization, is capable of being dissolved therein to an extent amounting to thirty-one per centum of the weight of such 105 solution. This caustic alkali solution thus modified by potassium acetate remains effective for mercerizing the cellulosic fibers

of a fabric into which viscose silk filaments have been incorporated and at the same time affords complete protection to such viscose silk against impairment of either its tensile 5 strength of its luster.

Except for the modification of the mercerizing caustic alkali solution suitable for ordinary mercerization by the addition thereto of any salt of an inorganic alkali base 10 which is soluble in such solution to an amount not much less than twenty per centum of the weight of that solvent and which is dissolved therein to the full extent of its solubility, the treatment of the fabric into 15 which cellulosic fibers of natural growth have been interwoven with viscose silk is in other respects substantially the same as that customarily employed in the mercerization of woven fabrics composed entirely of cotton, including the usual means and mode of applying tension thereto for the prevention of shrinkage.

Manifestly also by employing the same modified mercerizing solution as in the 20 treatment of woven mixed fabrics of the kind just specified, this invention may likewise be practised upon yarns or other unwoven fabrics which are composed partly of mercerizable cellulosic fibers, such as cotton or linen, and partly of viscose silk filaments and which in addition to their subjection to the action of such modified mercerizing solution are to be otherwise treated in the same manner as in the process of ordinary mercerization applied to similar 35 yarns or unwoven fabrics consisting entirely of mercerizable cellulosic fibers.

By way of further explanation it may be more explicitly stated that the caustic alkali 40 solution of standard strength for ordinary mercerization of natural cellulosic fibers usually consists of an aqueous solution of sodium hydroxid; that twenty-seven per centum of the total weight of this solution 45 is sodium hydroxid; that such solution has a density indicated by 60° of Twaddell's hydrometer; and that the extent of solubility of the respective soluble salts of the inorganic bases hereinabove referred to is estimated and intended to be specified in 50 percentage of the weight of the said standard mercerizing solution without regard to the specific gravity of any solution resulting from the introduction of either of those salts 55 into such standard solution.

Finally, it may here be particularly remarked that although the arsenites and arseniates of sodium, potassium and ammonium if employed to modify the mercerizing caustic alkali solution are sufficiently 60 soluble and effective therein to protect the viscose silk from practical deterioration in its tensile strength and degree of luster when intermingled with cellulosic fibers 65 which are subjected to the process of mer-

cerization; yet because of the well-known poisonous properties of arsenical compounds, precautions should be taken to wash out any residue of the alkali arsenite or arseniate left in the composite textile fabric 70 after treatment as aforesaid in order to render such fabric hygienically acceptable for the purposes of wearing apparel.

We claim:

1. The method of treating textile fabrics 75 composed of mercerizable cellulosic fibers intermixed with artificial silk filaments of viscose for the purpose of mercerizing such cellulosic fibers without practical injury to the viscose silk, by subjecting the composite 80 fabric thus constituted to a process of mercerization wherein the mercerizing solution of caustic alkali is modified by the addition thereto of a salt which has an inorganic base and which will not by reaction of the 85 caustic alkali therewith undergo change in its chemical composition, but which is soluble in the standard aqueous caustic alkali solution for ordinary mercerization to an 90 amount not much less than twenty per centum of the weight of such solvent, and is in fact dissolved to substantially the full extent of its solubility in the mercerizing caustic alkali solution employed in said process.

2. The method of treating textile fabrics 95 composed of yarn spun from mercerizable cellulosic fibers and interwoven with artificial silk filament of viscose for the purpose of mercerizing the fibers of such yarn without practical injury to the viscose silk, by subjecting the woven fabric thus constituted to a process of mercerization wherein the mercerizing solution of caustic alkali is modified by the addition thereto of a salt which has an inorganic base and which will 100 not by reaction of the caustic alkali therewith undergo change in its chemical composition, but which is soluble in the standard aqueous caustic alkali solution for ordinary mercerization to an amount not much 105 less than twenty per centum of the weight of such solvent, and is in fact dissolved to substantially the full extent of its solubility in the mercerizing caustic alkali solution 110 employed in said process.

3. The method of treating textile fabrics composed of mercerizable cellulosic fibers intermixed with artificial silk filaments of viscose for the purpose of mercerizing such cellulosic fibers without practical injury to the viscose silk, by subjecting the composite fabric thus constituted to a process of mercerization wherein the mercerizing solution of caustic alkali is modified by the addition thereto of a salt which has an inorganic alkali base and which is soluble in the standard aqueous caustic alkali solution for ordinary mercerization to an amount not much less than twenty per centum of the weight of such solvent, and is in 115 120 125 130

fact dissolved to substantially the full extent of its solubility in the mercerizing caustic alkali solution employed in said process.

5 4. The method of treating textile fabrics composed of yarn spun from mercerizable cellulosic fibers and interwoven with artificial silk filaments of viscose for the purpose of mercerizing the fibers of such yarn with-  
10 out practical injury to the viscose silk, by subjecting the woven fabric thus constituted to a process of mercerization wherein the mercerizing solution of caustic alkali is modified by the addition thereto of a salt  
15 which has an inorganic alkali base and which is soluble in the standard aqueous caustic alkali solution for ordinary mer-  
cerization to an amount not much less than twenty per centum of the weight of such  
20 solvent, and is in fact dissolved to substan-  
tially the full extent of its solubility in the mercerizing caustic alkali solution employed in said process.

5. The method of treating textile fabrics composed of cotton fibers intermixed with artificial silk filaments of viscose for the purpose of mercerizing such cotton fibers without practical injury to the viscose silk, by subjecting the composite fabric thus con-  
30 stituted to a process of mercerization wherein the mercerizing solution of caustic alkali is modified by the addition thereto of a salt which has an inorganic alkali base and which is soluble in the standard aqueous  
35 caustic alkali solution for ordinary mer-  
cerization to an amount not much less than twenty per centum of the weight of such solvent, and is in fact dissolved to substan-  
40 tially the full extent of its solubility in the mercerizing caustic alkali solution em-  
ployed in said process.

6. The method of treating textile fabrics composed of cotton yarn interwoven with artificial silk filaments of viscose for the purpose of mercerizing the fibers of such cotton yarn without practical injury to the viscose silk by subjecting the woven fabric thus constituted to a process of mercerization wherein the mercerizing solution of caustic alkali is modified by the addition thereto of a salt which has an inorganic alkali base and which is soluble in the stand-  
50 ard aqueous caustic alkali solution for ordi-

nary mercerization to an amount not much less than twenty per centum of the weight 55 of such solvent and is in fact dissolved to substantially the full extent of its solubility in the mercerizing caustic alkali solution employed in said process.

7. The method of treating textile fabrics composed of mercerizable cellulosic fibers intermixed with artificial silk filaments of viscose for the purpose of mercerizing such cellulosic fibers without injury to the viscose silk by subjecting the composite fabric thus 60 constituted to a process of mercerization wherein the mercerizing solution of caustic alkali is modified by the addition thereto of potassium acetate dissolved therein to substantially the full extent of its solubility. 70

8. The method of treating textile fabrics composed of yarn spun from mercerizable cellulosic fibers and interwoven with artificial silk filaments of viscose for the purpose of mercerizing the fibers of such yarn 75 without injury to the viscose silk, by sub-  
jecting the woven fabric thus constituted to a process of mercerization wherein the mer-  
cerizing solution of caustic alkali is modi-  
fied by the addition thereto of potassium 80 acetate dissolved therein to substantially the full extent of its solubility.

9. The method of treating textile fabrics composed of cotton fibers intermixed with artificial silk filaments of viscose for the 85 purpose of mercerizing such cotton fibers without injury to the viscose silk by sub-  
jecting the composite fabric thus constituted to a process of mercerization wherein the mercerizing solution of caustic alkali is 90 modified by the addition thereto of potas-  
sium acetate dissolved therein to substan-  
tially the full extent of its solubility.

10. The method of treating textile fabrics composed of cotton yarn interwoven with 95 artificial silk filaments of viscose for the purpose of mercerizing the fibers of such cotton yarn without injury to the viscose silk, by subjecting the woven fabric thus constituted to a process of mercerization 100 wherein the mercerizing solution of caustic alkali is modified by the addition thereto of potassium acetate dissolved therein to sub-  
stantially the full extent of its solubility.

SAMUEL MANSFIELD JONES.  
IVAN OTHMA HARLOW.